

# United States Patent

[11] 3,581,690

[72] Inventor **G. Claudio Zapata**  
Mexico City, Mexico  
[21] Appl. No. **785,443**  
[22] Filed **Dec. 16, 1968**  
[45] Patented **June 1, 1971**  
[73] Assignee **Zapata Industries Inc.**  
Frackville, Pa.  
Continuation-in-part of application Ser. No.  
731,852, May 24, 1968, now abandoned.

[56] **References Cited**  
UNITED STATES PATENTS  
3,257,021 6/1966 Brockett..... 215/39  
3,233,770 2/1966 Waters ..... 215/40  
3,361,281 1/1968 Kehe ..... 215/39  
1,170,160 2/1916 Ingram et al. .... 215/39  
2,620,939 12/1952 Weisgerber ..... 215/40  
*Primary Examiner*—Richard J. Herbst  
*Assistant Examiner*—Michael J. Keenan  
*Attorney*—Pennie, Edmonds, Morton, Taylor and Adams

[54] **CROWN TYPE CLOSURE WITH DOUBLE REMOVABLE LINER UNIT ENCLOSING TRAPPED INDICIA AND METHOD OF MANUFACTURE**  
6 Claims, 3 Drawing Figs.  
[52] U.S. Cl. .... 113/80, 113/121  
[51] Int. Cl. .... B21d 51/46  
[50] Field of Search. .... 113/121 A, 121 AA, 121 B, 121 F, 116 BB, 80, 80 C, 80 D, 80 DA; 215/39, 40

**ABSTRACT:** The closure cap or crown for bottles disclosed, comprises a crown shell having a print covered by a size coat, a removable liner unit including a first removable liner coating in the shell over the size coating carrying printed indicia, such as a question, and being either transparent or opaque, a second liner coating of transparent plastic material covering the first liner coating and the printed indicia thereon, and an annular sealing ring at the periphery of the second liner coating.



PATENTED JUN 1 1971

3,581,690

FIG. 1



FIG. 2



FIG. 3



INVENTOR.

Claudio Zapata G.

BY

*Paulie, Edwards, Morton, Taylor & Co.*

ATTORNEYS

**CROWN TYPE CLOSURE WITH DOUBLE REMOVABLE LINER UNIT ENCLOSING TRAPPED INDICIA AND METHOD OF MANUFACTURE**

**Cross-Reference to Related Application**

This application is a continuation-in-part of the applicant's pending U.S. application Ser. No. 731,852, filed May 24, 1968, now abandoned.

**BACKGROUND OF THE INVENTION**

**1. Field of the Invention**

This invention relates to improvements in bottle cap closures, particularly crown-type closures provided with a removable liner unit of plastic material carrying selected printed indicia and seated over an interior size coating of the closure.

**2. Description of Prior Art**

Prior disclosures relating to the above subject comprise U.S. Pat. Nos. 3,233,770, 3,361,281, and 3,257,021. These patents were granted recently, and the first discloses a crown-type closure provided with a removable liner which is arranged to carry printed indicia which may be mailed out by a customer to the distributor or manufacturer. In this instance the liner is a clear plastisol material. The crown closure is provided with a coating of lacquer and indicia are printed on this lacquer in the interior part of the closure. Subsequently, the liner is applied over the printed indicia material. In this construction the relationships are such that the lacquer coating is nonadherent to the liner, and the printing is selectively adherent to the liner, so that it is removed from the closure with the removable liner. The patent describes specific vinyl chloride polymer plastisols and plasticizers and other materials which may be used in forming the films and coatings of the present invention.

The third patent referred to above has a disclosure very similar to the first. In this instance the printed indicia are printed on the lacquer of the closure and covered over with a transparent elastic cushion liner, so that the printing is visible therethrough when looking into the closure. The liner may be peeled from the closure and carry the printed indicia adhering thereto because of its preferential adherence to the liner rather than the lacquer on the closure. To begin with, the indicia is adherent to both the lacquer and the liner but the adhesion between the indicia and the liner is said to be greater than that between the indicia and the lacquer.

In these prior disclosures the printing material used to form the indicia are said to reduce the adhesion between the liner and the lacquer over a considerable portion of the area of the closure. Overbaking of the lacquer is also disclosed.

The attempt to remove the printed indicia in the prior art disclosures, along with the removable liner, is in many instances only partially successful. Sometimes there is only a partial transfer of the indicia to the liner when it is removed from the closure and in a number of instances a poor or illegible image or printing results. According to the present invention, the removable liner unit provides the indicia or image in the perfect condition in which it is printed. This is achieved by providing a first plastic coating over the lacquer or sizing, and any printing thereon, on the interior of the shell under conditions so that it is readily removable. Next, this first coating or film is printed by the various procedures described in the above patents to provide the desired indicia. After printing the first film, a second film is applied to the first film over the printing, so that the latter is trapped between the two films and kept in perfect condition until, during and after the liner unit is removed from the closure.

One of the objects of the present invention is to achieve good promotional features without sacrificing the functional properties of a plastic lined crown. An "easy-removal" liner manufactured by sacrificing the normal adhesion between the liner and crown shell frequently results in blister formation in the central panel caused by gas diffusion from the bottle. Such blisters are objectionable in appearance and can lead to a

distortion of the gasket ring and subsequent loss of pressure retention.

In prior attempts to achieve easy removal by using the thumbnail to remove the plastic liner from the sheet, the above functional features were sacrificed by either providing a low order of adhesion of the liner to the shell (U.S. Pat. No. 3,257,021) or only adhering the liner in selected areas (3,233,770). In each case, the reduction in adhesion between liner and shell to accomplish "easy removal" results in an occasional loose liner in the shell, blister formation, gas leakage, or difficulty in removal by thumbnail because the reduction in adhesion is difficult to control.

**SUMMARY OF THE INVENTION**

The present invention comprises a container closure provided with a size coating which may be printed, and a removable liner unit as described above, which includes first and second films or coatings between which indicia are trapped.

20 This liner is prepared and formed in such a way along with an annular seal that it provides protection for the goods sealed in the container and at the same time provides a readily removable liner unit after the closure is removed from the container.

In accordance with the invention, large tinned steel sheets 25 of the type used in this art, shown and described in U.S. Pat. No. 3,257,021, are printed then coated with a low solids size coat. This is the initial lacquer coating of the large tinned sheets, after which that coating is baked on at a temperature to give good adhesion to the tinned sheet and printing. This 30 size coating, at the positions within the sealing rings, is now advantageously printed with some message, such as a question or answer, for example with printing ink material.

As an additional novelty to aid in easy removal of the liner 35 unit without sacrificing functional properties, a ring of clear ink can be printed on the interior size coating around the gasket areas to reduce adhesion of the liner unit to the sizing, thus facilitating easy removal with an average fingernail. This ring of clear ink may be used or not depending on the ease of 40 removal required.

The second coating referred to as the first film of the removable liner unit is applied over the large sheets on the size coating and on the ring of clear ink. This coating is preferably 45 a polyvinyl chloride organisol applied to produce a heavier film weight than the size coat. It may be transparent but in some instances it is made of opaque material. The next step is the printing of an image or indicia on the large sheet in the 50 positions of the respective closures to be stamped from the sheet. This goes on the second coating and the printing is preferably effected by a printing ink of known type applied in various ways, such as by screen or lithographic press, and may be trail coated with the third coating, or a third, transparent coating, may be applied over the second coating and adhered to it. Each coating is heated or baked before the application of 55 the next coating, and the third coating is also baked.

The conditions are such as to control the adhesion, particularly between the size coating and the second coating. If the 60 third coating is applied, the large sheets are subjected to the usual punching operation to cut out and form the crowns, each of which would carry the three coatings with the various indicia and/or the clear ink ring. In this case the crowns are finally provided with an annular sealing gasket of a foamed or solid polyvinyl chloride plastisol material of known type, and the annular seals are baked and cured in an oven. Instead of 65 applying the third coating as above, an advantageous structure is provided by simultaneously applying a third coating and annular sealing ring. This third coating and sealing ring are applied to the punched out crowns by a cold punch die operation 70 on hot plastic material. No curing is thereafter necessary. The plastic material used is such that the area inside the sealing ring is transparent.

In carrying out the main features of the invention some 75 modifications may be made, for example, the crowns may be punched out following the printing of the indicia on the

second coating after which a transparent film is provided, for example, by spinning in a center panel section to cover a limited area short of the edge of the panel. An annular seal may then be applied in each closure, so that it covers the peripheral edge of the second film and is adhered to the first film of the removable liner.

#### BRIEF DESCRIPTION OF THE DRAWINGS

The drawing provided herewith as a part of this application illustrates the invention in connection with two embodiments.

In the drawing:

FIG. 1 comprises an enlarged broken sectional view through a crown-type closure comprising one embodiment having a removable liner with trapped indicia over a ring of release material, although it may be without the ring of release material, and an annular seal constructed and arranged in accordance with the invention;

FIG. 2 is a view similar to that of FIG. 1 showing a second embodiment provided with a removable liner, located over indicia under the size coating, and containing trapped indicia in which the transparent third film and annular seal are integral; and

FIG. 3 is a plan view showing a removed liner message unit and crown according to FIG. 2.

#### DESCRIPTION OF THE PREFERRED EMBODIMENT

In both FIGS. 1 and 2 the crown closure or bottle cap comprises a rigid tinned steel plate member 10. The outside of the crown closure is provided with a size lacquer coating 12 called a modified vinyl size coating of known type on which the usual exterior printing is applied. Inside the crown there is also a modified vinyl or primer size coating 14 covering the entire interior surface of the shell including the corrugated skirt 16.

In FIGS. 1 and 2 the various coatings are cut back to expose a part of the coating beneath. The removable liner unit is applied over the size coating 14 and consists of a coating 18, a somewhat heavier coating than that of the coating 14. These coatings may be applied over the entire interior area of the crown, including the corrugated skirt portion 16. The coatings 14 and 18 are applied uniformly over the large sheets before the crowns are punched therefrom. However, the coating 18, of similar material to the coating 14, is applied in such a manner as to apply limited adhesion to the size coating 14.

The limited adhesion of the coating 18 to the size coating 14 can be greatly reduced by applying a ring of clear ink 15 to the size coating 14 at the position below the sealing ring gasket of the crown. This reduces the adhesion under the gasket area and thus facilitates easy removal with the average fingernail. The clear ink used may comprise a property which is designed to cause the ink to adhere selectively to the size coating 14 only. Easy removal may also be effected by providing a ring of printed indicia at the position of the ring layer 15, using the same type of ink but preferably one which is not clear but which is made visible such as an answer to a question when the removable liner unit is finally removed from the crown.

Additional printing 19 is applied to the tinned steel plate 10, before applying the size coating 14, in the area inside that of the ring 15. This printing may be an answer to a question and as illustrated comprises the answer shown in FIG. 3, FIG. 1 showing the lettering "THE ST." The lettering may be in a desirable color and since the printing is trapped under the size coating it will not adhere to the coating 18. In this case the coating 18 would be made of opaque material, so that the printing under the interior area of the transparent size coating will only be made visible when the liner unit is removed. This is described more in detail in connection with FIG. 2.

Following the application of the printing 19, coating 14, the ring 15 and the coating 18, the large sheets are printed at the locations of the crown panels to provide the desired indicia or message on the panel section of the coating 18. Such indicia is indicated at 20 which for purposes of illustration may be a question as in FIG. 3, or comprise the letters "SODA" which may be only a part of the message.

In the embodiment in FIG. 1 the crowns may be punched from the large sheet after applying the printing 20 and thereafter each crown is provided with a transparent liner film 22 by spinning the crowns and applying a blob of polyvinyl chloride plastisol or organisol material to the center of the panel portion so that it spreads out thinly to the periphery of the panel portion 24 of the crown. This film coating 22 completely covers the printed indicia 20 and its periphery is adhered firmly to the coating 18. Finally, the crowns are slowly rotated while a sealing ring 26 is applied over the peripheral portion of the film 22 above the element 15. The various coatings and the sealing ring 26 are subjected to baking operations described more in detail hereinafter. The transparent coating 22 may extend completely to the skirt of the crown or only to a position so that its edge is well covered by the sealing ring 26 or as shown in FIG. 1. The film or coating 22 may be spun in, or applied as spots by screen printing, or spot coating on the large sheet before punching.

The embodiment illustrated in FIG. 2 may include elements corresponding to the elements shown in FIG. 1 up to and including the printed indicia material 20' on the coating 18. In this view, the sealing ring and the center panel coating are applied as a single integral element which comprises a central transparent film panel 22' molded integrally with a ring gasket 26'. The material used in making these two elements comprises a dry blend gasket molding liner material of known type supplied to the crowns hot and molded with a cold die. The integral element includes a peripheral portion 28 immediately outside the gasket 26' and this portion together with the area beneath the gasket is firmly adhered to the coating 18.

In the construction shown in FIG. 2 an adhesion reducing layer 15' similar to the layer 15 of FIG. 1 can be provided on the size coating 14 beneath the area covered by the sealing ring 26' and the peripheral portion 28. Printed indicia 21, illustrated by the letters C and O are also provided on the layer 15' to form an entire ring of indicia which is also of adhesion reducing material. This indicia is made visible when the removable liner is taken from the crown.

The crown and removable liner shown in FIG. 2 are provided with the indicia set out in FIG. 3. For example, the indicia 20' is printed on the coating 18 within the panel area inside the ring 26'. Since the layer 22' is transparent the question of the indicia 20' is plainly visible before the removable liner is taken from the crown. In this instance the coating 18 is preferably opaque so that the answer of the indicia 30 located under the size coating 14 is not disclosed until the removable liner is pulled out of the crown.

The removable liner shown in FIG. 3 may have the structure illustrated in either FIG. 1 or FIG. 2, but FIG. 3, for purpose of simplification, does not include a showing of the element 15 of FIG. 1 or the elements 15' or 21 of FIG. 2.

In producing the combination illustrated in FIGS. 2 and 3, the indicia or answer 30 is printed on the tinned sheets 10 and cured before applying the size coat 14. Following this, the coating 18 is applied over the size coating 14 and the elements 15' and 21 thereon. This coating is cured, after which the indicia of the question 20' is applied, following which the large sheets are passed through a curing oven at from 30° to 335° F. for a period of about 10 minutes. The coating 18 is preferably opaque, so that the answer indicia 30 on the tin is not visible or learned until the removable liner is taken from the crown.

The layer 22' and the ring seal 26' are applied over the question indicia 20' in the manner described above. It is to be understood, of course, that instead of the integral layer 22' and ring 26', one may use the coating 22 and sealing ring 26.

#### EXAMPLE

The large tinned steel sheets, from each of which a considerable number of crowns are finally punched (as in U.S. Pat. No. 3,257,021) are printed with indicia 19 or 30, later coated with a commercial polyvinyl chloride liquid sizing material following which the large sheets are baked in an oven

at a temperature of from approximately 395° to 405° F. for a period of approximately 10 minutes. The coating 14 may amount to approximately 4 to 8 mg. per 4 square inches of the sheet and the baking cures and hardens the size coating 14, so that it is adhered firmly to the tin coat of the steel sheets and yet gives an outer surface which has limited adhesion characteristics with respect to subsequent coating 18, when coating 18 is baked at temperatures below the fusion point of the two coatings.

Prior to applying the coating 18, the sizing coat 14 can receive the ring of low adhesion material 15 or 15' and printing 21 is applied to the ring or band 15'. The lacquered or sized sheets are thereafter coated with the plastic film 18, which has a high solids content commercial coating material sometimes referred to as polyvinyl chloride organisol, examples of which are given in the above patents. This coating amounts to 25 to 70 mg. per 4 square inches and is baked on in an oven at a temperature of from 325° to 345° F., preferably 335° F. In the oven the sheets are passed along at a rate such that a baking time of about 10 minutes is obtained and the temperature and time of baking are adjusted to provide some adhesion to the sizing coat 14, but an adhesion which is limited. A good film 18 is obtained with 20 to 25 mg. per 4 square inches.

The next step of the process is that of printing an indicia message or question on the exposed surface of the cured coating 18. The indicia 20 and 20' are applied in a known manner by the use of a suitable printing ink material, such as disclosed in said patents, preferably by an offset litho method. The printing of an entire sheet at a time with the multiplicity of locations is accomplished in a very accurate manner by this method. However, the printing may be accomplished by ordinary offset procedure, lithographic gravure, silk screen or flexographic methods. The printed sheets are baked at a temperature of from 295° to 305° F. for a period of about 10 minutes to fix and cure the printing material. Printing 19 and 30 may be cured by the same procedure before applying the size coating 14.

In accordance with the embodiment shown in FIG. 1, the fourth step is the provision of a solid coating film 22 over the indicia 20 and the remainder of the coating 18 to the extent shown. This film is applied either to the sheets or to the individual crowns after they are punched from the sheets as described above.

The transparent film coating 22 may be applied to the individual crowns over the indicia 20 and the coating 18 to the extent shown by depositing a blob of polyvinyl chloride organisol into each crown and rotating it until the coating 22 spreads out. The coating 22 either on the sheets or the crowns is baked at a temperature of from 305° F. to 325° F., preferably 315° F. for a period of about 10 minutes and adhered to the coating 18. The plastisol used to form the film 22 produces a clear film through which the question or other indicia 20 are visible.

Finally, the foamed plastisol gasket 26 is applied in each crown on top of and adhered to the peripheral portion of the film 22. The material used for this gasket is a commercial product and is applied in the ring shape, in a known manner, while slowly rotating the crown. The gasket is baked in the crown at a rather high temperature, that is, 390° F. to 400° F. for a period of 1 minute. Known types of baking ovens may be used in effecting the various baking steps.

The procedure followed with respect to the embodiment shown in FIGS. 2 and 3, after the indicia are printed on the film 18 comprises the use of a cold-molded liner comprising the transparent film layer 22' and the raised ring gasket 26' which are molded in one piece. The liner may be cold die molded from a hot molten pellet of commercial polyvinyl chloride liner material. The heat in the molten pellet being molded, causes fusion between the formed liner material and the film 18, instantaneously, that is, during only a fraction of a second.

It is to be understood that the film 22' and the integral ring gasket 26' are one piece, and may be applied in a known manner by the use of a cold molding plunger pressed downwardly on a suitable quantity of hot molten commercial polyvinyl chloride liner material, which may originally be a dry blend.

In accordance with the invention the separation of the film 18 from the size or lacquer coating 14, and the elements 15, 15' and 21 when the removable liner unit is removed from the closure, is achieved because of the control of adhesion. The coating 14 is a vinyl size coating as used in the industry, which adheres well to the tin plate and elements 19 and 30 under the conditions described in the above example, while the coating or film 18 is of the modified polyvinyl organisol type, or dispersion of polyvinyl chloride in a plastisol with other modifying resins. This material has the property to develop only a physical adhesion to the vinyl size coating and little if any adhesion to the elements 15, 15' and 21, under the baking conditions described in the above example. It is baked at a temperature below 350° F. at which it does not develop maximum chemical adhesion with the size coating or the mentioned elements. The size coating 14 is baked at a normal baking temperature which gives good adhesion to the tin plate and provides low adhesion surface for the coating 18.

When a bottle cap, for example, is removed from a beverage bottle by a customer, the liner unit is readily removable from the size coating 14 by breaking the thin film 18 partly around the outside of the gasket 26 along the dotted line *a-a*. This may be accomplished readily by a fingernail or pen knife. When the liner is lifted at one point, a separation occurs between the film coating 18, the size coat 14 and elements 15, 15' and 21. Since the printed question or message indicia 20 or 20' is located on the film 18 and trapped by the film 22, the indicia is removed with the liner message unit, which has been sealed away from the contents of the container, the lacquer coating 14 and the printing 19 and 30.

In FIG. 2 the message liner unit is readily removable by running a fingernail or a pen knife along the dotted line *a-a* and edge of film portion 28. This severs the film 18, so that the sealed message or question unit is readily removable from the size coating 14 and the elements 15' and 21.

The closures or crowns of the present invention may be of the press-on or screw-on type for use on soft drink or other bottles, jars and other containers.

An excellent product can be made without making use of the size coating 14. Therefore, the coating 18 may be applied directly over the indicia 19 or 30 as well as the elements 15, 15' and 21, which would be applied directly to the tinned surface of the steel plate 10. In this construction the printing 19, 21 and 30 may be omitted so that a single message unit is provided which is sealed between the films 18 and 22 or 22'.

I claim:

1. In a method of making container closure caps of the type including a rigid shell provided with an adherent size coating on its inner surface, and a removable plastic sealing liner unit releasably secured to the size coating in the interior of the rigid shell, wherein the improvement comprises the steps of applying and curing a size coating on one surface of a sheet of material for making a multiplicity of closure caps, applying and curing a plastic coating film over said size coating, printing indicia on the film on said sheet at the locations for the caps, curing the printed indicia on said film, punching the closure caps from the sheet, applying and curing a transparent plastic coating film and integral sealing ring over the printed indicia and on the film on which it is located in each cap and adhering it thereto thereby trapping the printed indicia between said films, whereby caps are produced having readily removable liner units comprising indicia trapped and protected between the two films.

2. A method as claimed in claim 1, including the step of curing the size coating by baking it at a temperature of from 395° to 405° F. for a period of about 10 minutes to give its outer surface of low adherent quality with respect to the plastic coating applied thereover when cured.

3. A method as claimed in claim 2, wherein the plastic coating applied over the cured size coating is baked and cured at a temperature of from 300° to 345° F. over a period of about 10 minutes.

4. A method as claimed in claim 1, including the step of printing indicia on said surface of the sheet of material at the locations of the shells prior to the step of applying the size coating, and wherein the plastic coating film over the size coating and over the said indicia is opaque and nonadherent to

10

said size coating, whereby said indicia is made visible only after removing the liner units from the completed caps.

5. A method as claimed in claim 1, including the step of applying a ring of nonadherent material on the cured size coating directly beneath the position of the sealing ring.

6. A method as claimed in claim 5, wherein the ring or low adherent material is in the form of printed indicia made visible only after the liner unit is removed from the cap.

15

20

25

30

35

40

45

50

55

60

65

70

75

UNITED STATES PATENT OFFICE  
CERTIFICATE OF CORRECTION

Patent No. 3,581,690 Dated June 1, 1971

Inventor(s) Claudio Zapata G.

It is certified that error appears in the above-identified patent and that said Letters Patent are hereby corrected as shown below:

Title page, line 1, change the inventor's name to  
--Claudio Zapata G.--.

Column 8, line 6, (claim 6, line 1) change "or"  
to --of--.

Signed and sealed this 25th day of April 1972.

(SEAL)

Attest:

EDWARD M.FLETCHER, JR.  
Attesting Officer

ROBERT GOTTSCHALK  
Commissioner of Patents